

July 28, 1925.

1,547,616

C. A. SCHARSCHU

## MAGNETIC MATERIAL

Original Filed Dec. 27, 1920

Fig. 1.



Fig. 2.



Fig. 3.



Inventor:  
Charles A. Scharschuh,  
by *Albert J. Davis*  
His Attorney.

## UNITED STATES PATENT OFFICE.

CHARLES A. SCHARSCHU, OF PITTSFIELD, MASSACHUSETTS, ASSIGNOR TO GENERAL ELECTRIC COMPANY, A CORPORATION OF NEW YORK.

## MAGNETIC MATERIAL.

Original application filed December 27, 1920, Serial No. 433,147. Divided and this application filed April 7, 1922. Serial No. 550,435.

To all whom it may concern:

Be it known that I, CHARLES A. SCHARSCHU, a citizen of the United States, residing at Pittsfield, in the county of Berkshire, State of Massachusetts, have invented certain new and useful Improvements in Magnetic Material (being a division of my application, Serial No. 433,147, filed December 27, 1920), of which the following is a specification.

10 The present invention comprises an improved magnetic material and in particular silicon steel capable of utilization at high efficiency in varying magnetic fields.

In the construction of cores for electrical apparatus, especially of the alternating current type, such as transformers and dynamo-electric machines, it is highly important to use magnetic material in which the watt losses, due to hysteresis and eddy currents, 20 are as low as possible. Consequently efforts have been made during the development of the electrical industry to improve the magnetic properties of core material, and the substitution of silicon-iron and other alloys for ordinary steel has indeed effected a considerable saving in electrical energy. Efforts to further improve the magnetic properties of silicon steel have been and are being made by manufacturers of this 30 material since it is realized that a reduction of core loss by even a small percentage results in the saving of a large amount of energy; thus a reduction of core loss of one or two per cent is looked upon as an important achievement.

Silicon steel usually contains from 3.75% to 4% silicon and about .07 per cent carbon; it is ordinarily made in the open hearth furnace; it is cast into ingots and these are rolled into thin sheets which are used in core construction. The open hearth process results in a material in which a considerable amount of slag is distributed throughout the mass in which the sulphur content is generally 40 as high as from 0.03 to 0.04 per cent. I have found that the impurities carried by the slag and especially the high sulphur content of the product are detrimental characteristics of the magnetic material, since to their presence a large percentage of the hysteresis action is due.

I have discovered that when magnetic

material of any kind, and especially silicon steel, is made substantially free of slag inclusion and the sulphur content is reduced to and below .010 and usually as low as 0.005 per cent and even lower; that in such material the core loss is remarkably reduced, the reduction amounting on the average to about 12 per cent and is in individual cases still greater.

I have made claims herein on a new magnetic material having the above characteristics. In the application from which this application has been divided and which has matured into Patent No. 1,487,275, of March 18, 1924, claims have been made on a process of making my improved material which consists in treating the material in a fluid state whether it be scrap or when already fused by the open hearth process, in such manner as to exclude the admission of air; expel the occluded particles of slag from the interior of the fused mass to the surface and then pour the material from underneath the sheet of slag which usually is formed on the surface.

This process is preferably carried out by the use of an induction furnace of a specific construction which constitutes a part of my invention. While the fused mass is in the induction furnace and preparatory to the practice of my invention, the material may be chemically refined in any ordinary or improved manner.

In the accompanying drawing, Fig. 1 illustrates partly in elevation and partly in vertical section an induction furnace embodying structural features of my invention; Fig. 2 is a plan view of the furnace chamber, the furnace top being removed; and Fig. 3 is a top view, the primary coil and housing being shown in part broken away.

The induction furnace shown in the drawing comprises an annular furnace crucible 1, surrounding a magnetic core 2, which has a flat primary winding 3, supplied with alternating current by conductors not shown. The primary winding may consist of annular sections, as shown; it is suitably mounted on a framework 4 above the crucible 1, in the manner set forth in Patent No. 1,326,120 to Unger. The furnace crucible is provided with a refractory lining 5, which is in di-

rect contact with the body of metal 6 to be melted, and consists preferably of particles of highly sintered or fused magnesia molded with a binder such as magnesium sulphate 5 to form a solid mass. This lining rests upon a wall of refractory brick 7, which in turn is supported by a suitable casing 8, made of boiler plate or the like. I have discovered that the location of the channel 10 or crucible 1 beneath the primary winding 3 subjects the molten mass in the crucible, constituting the secondary in the induction furnace, to the action of an alternating electro-magnetic field in such a manner that 15 the slag particles occluded in the fused mass tend to separate from the metal, as will be hereinafter more fully explained.

The crucible 1 is provided with a refractory cover 9 which may consist of wedge-shaped sections, as shown in Fig. 3. The primary winding is preferably supported 20 and surrounded by a shell 10 containing ventilating openings 11, but I wish it to be understood that these and other structural 25 details are shown merely for the purposes of illustration.

The pouring spout 12 communicates with the furnace chamber near the bottom like the spout of a teapot, so that the fused 30 metal may be poured from the furnace from beneath the top slag layer without causing this slag or any part of it to be mixed with the metal. The pouring spout is provided with a door 13. The charge 35 receiving opening 14 is similarly provided with a door (not shown). A pouring spout of this character has heretofore been suggested for use in another kind of furnace, but in the induction furnace used for the practice of my process it cooperates with the magnetic function of the apparatus to assist the removal of the occluded slag particles.

The metal to be refined may be received in a molten state from any suitable source, for example, a Bessemer converter, an open hearth furnace, or an arc furnace, and may consist of soft steel, hard steel, or any alloy steel. My invention is also applicable to the melting of cold material either as scrap or new material directly in the induction furnace. The metal is allowed to attain a temperature of about 75° to 150° C. in excess of its melting point and is maintained in that condition for a period of from 45 minutes to one and one-half hours in addition to the time required for chemical refinement if such is resorted to while the metal is in a fluid state in the induction furnace.

When the induction furnace is charged with scrap or raw material, the ordinary chemical refinement is practiced right there, and after the refining slag has been removed in the ordinary manner a new slag is added.

This is preferably a basic slag consisting, for example, of lime and silica, the latter not exceeding 20%, and in some cases a small amount of fluorspar is added to thin the slag. Any other suitable slag which is 70 basic in character may be used when chemically refined molten metal from any source, such as a Bessemer converter, an open hearth furnace or an arc furnace is introduced into the induction furnace, the same 75 procedure is observed, that is to say, a basic slag of the general character above indicated is added.

The molten metal is subjected to the electro-magnetic purifying treatment which I 80 will now describe in greater detail. Owing to the location of the primary winding above the crucible element of the furnace, the alternating flux gives to the molten mass a slow but powerful movement from the 85 inner edge of the annular channel downwardly toward the bottom and upwardly along the outer edge of the channel. In this respect the action of the flux upon the fluid metal is different from that of the 90 magnetic flux when the primary winding is concentric with the channel, for in the latter case the molten metal is violently agitated in an irregular manner, causing the 95 occluded slag particles to mix continuously with the metal and effectually preventing a separation of the same. By locating the primary winding above the crucible channel, the movement of the metal becomes very 100 much slower. There are two forces acting on the molten charge tending to expel the slag from the metal, namely, the compressive effect of the magnetic field upon the charge and the electro-dynamic effect which exerts 105 a different repellent action upon the slag 110 and metal.

The compressive or pinch force of the magnetic field of a current-carrying conductor is a force acting radially inward upon the current-carrying elements of the conductor. As the slag is a poor conductor it tends to be squeezed out somewhat like water being squeezed out of a sponge. The separating action due to the electro-dynamic effect 115 is somewhat comparable to the separation occurring in a centrifugal separator. The current-carrying metal is repelled with greater force than the slag particles. As the magnetic field is applied from above, the slag particles tend to come to the surface. Due to the combined effect of the slow and regular movement of the charge and the 120 expulsive force exerted on the slag particles, they are carried with the metal to the surface and there attach themselves to the slag. In this manner the fused mass is substantially freed from slag occlusion.

My improved form of pouring spout 12 which communicates with the bottom of the crucible 1 prevents the remixing of the metal 125

with the expelled slag when the metal is poured by tilting the furnace, so that the advantage of the preceding melting treatment under the influence of the electromagnetic field is not lost when the metal is poured.

The material thus made, in contact with furnace gases, may be distinguished from a vacuum-fused product by the fact that it contains a substantial amount of gas. Silicon steel made in accordance with my invention has been found by analysis to contain about 1000 to 2000 cubic centimeters of gas per kilogram of metal. This gas consists largely of hydrogen together with small amounts of carbon dioxide, carbon monoxide and nitrogen.

The carbon content of the material is substantially unaffected by the refining treatment in the induction furnace.

What I claim as new and desire to secure by Letters Patent of the United States is:—

1. An electromagnetic structure of ferrous material, having a sulphur content less than 0.01 per cent by weight and containing gas in a quantity characteristic of metal fused in contact with furnace gas at atmospheric pressure, said material being capable of operating as a core in an alternating magnetic field with a materially low-

er energy loss than similar material having a higher sulphur content.

2. A ferrous magnetic material containing silicon as an alloying element, having a carbon content substantially no lower than ordinary open hearth silicon steel, having a sulphur content substantially no greater than 0.010 per cent, and being characterized by a substantial gas content which is materially higher than the gas content of similar material fused in a vacuum, said material being capable of operating in an alternating magnetic field with materially lower energy loss than similar material having a higher sulphur content.

3. A magnetic material consisting largely of iron, containing about 3.75 to 4 per cent silicon, about 0.07 per cent carbon, not substantially more than 0.005 per cent sulphur, and having a gas content of more than about 1000 to 2000 cubic centimeters per kilogram, said material being capable of operating in an alternating magnetic field with a materially lower energy loss than similar material having a substantially higher sulphur content.

In witness whereof, I have hereunto set my hand this 5th day of April, 1922.

CHARLES A. SCHARSCHU.